

July 17, 1923.

1,462,220

C. WIEGANDT

LABEL

Filed Feb. 6, 1923

Fig. 1



Fig. 2



Inventor:

Carl Wiegandt  
by

Fritz Koennecke  
Attorney.

## UNITED STATES PATENT OFFICE.

CARL WIEGANDT, OF BARMEN, GERMANY, ASSIGNOR OF ONE-HALF TO ALBERT VIEHMANN, OF BARMEN, GERMANY.

## LABEL.

Application filed February 6, 1923. Serial No. 617,291.

*To all whom it may concern:*

- Be it known that I, CARL WIEGANDT, a citizen of the German Empire, residing at Barmen, Germany, have invented certain new and useful Improvements in Labels, for which I have filed an application for patent in Germany on December 13, 1920, and of which the following is a specification.
- 10 My invention relates to labels made of sheet-metal, especially sheet-iron, which may be fastened to packages, such as bags, bales, chests or the like, by tying or nailing up.
- 15 The essential feature of my invention consists in this that the label is coated with an ordinary light-coloured oil-paint containing hydrochloric acid or an equivalent medium. To this paint ordinary writing ink
- 20 as well as ordinary printing ink will firmly adhere so that the coated label may be written on and printed.

The new label is distinguished from the known sheet-metal labels which are lined with paper by the great durability of the coating of paint, the same notwithstanding also the influence of wetness so that the address or other superscription applied to the label can not get lost. Furthermore, in consequence of the fact that the coating of paint prevents oxidation of the surface of the sheet-metal, obliterating of the address by rusting or the like is entirely avoided. Finally by the admixture of hydrochloric acid to the oil-paint the result is obtained that writing and printing inks adhere not only to the surface of the coating, but penetrate into the latter yet without dispersing. Thus the lasting of the address or other superscription applied to the label is greatly increased, the address or the like can be neither washed away nor blurred.

The coating capable of being written on or printed may be provided either on one or on both sides of the label. In the latter instance the label can be used twice. When the label consists of ordinary sheet-iron and only one side is coated with a paint of the kind above referred to I prefer to protect the other side of the label against oxidation by coating it with a colourless varnish or any other cheap coating medium.

The label may have any known or desired shape, and it may, as usual, be fitted with fastening holes or eyelets.

My new label is, by way of example, illustrated on the annexed drawing in which:

Fig. 1 is a front view of the label, and

Fig. 2 is a sectional elevation on the line 2—2 of Fig. 1 drawn on an enlarged scale. <sup>60</sup>

The label shown consists of a rectangular plate *a* of sheet-metal, ordinary sheet-iron for example, the same being at its front-side provided with a light-coloured, preferably white coating *b* of oil-paint or lake <sup>65</sup> capable of being written on and printed with ordinary writing and printing ink. At the back-side the label is coated with a colourless varnish or other cheap coating medium *c*, which only prevents oxidation. <sup>70</sup> In the vicinity of the lateral edges the label is fitted with the usual fastening holes or perforations *d* which may be edged with eyelets *f*.

The coating *b* may consist of any ordinary oil-paint or lake to which a suitable quantity of hydrochloric acid is added. The following composition has proved particularly useful:

2 parts of linseed oil,  
5 parts of zinc-white,  
6 parts of petroleum benzin,  
1 part of hydrochloric acid.

This composition results in a light, mat coating which can easily be written on or printed with ordinary writing and printing ink and which sucks up the said ink without causing the same to disperse which would, of course, render the address or other superscription more or less illegible. <sup>85</sup> <sup>90</sup>

I wish it to be stated that my invention is not restricted to the precise embodiment shown and described for many alterations and variations may suggest themselves to those skilled in the art without departing from the spirit of my invention as pointed out in the claims. <sup>95</sup>

## Claims:—

1. As a new article of manufacture: a label made of sheet-metal and coated with <sup>100</sup> an ordinary light-coloured oil-paint containing hydrochloric acid.

2. As a new article of manufacture: a label made of sheet-metal and coated with a composition of linseed oil, zinc-white, and <sup>105</sup> hydrochloric acid.

In testimony whereof I affix my signature.

CARL WIEGANDT.